

March 5, 1957

E. N. MAISEL

2,784,132

AIR PERMEABLE FIBROUS BATT

Filed May 11, 1953



Inventor:

Emanuel N. Maisel,  
By: Schneider & Dressler, Atty.

1

2,784,132

## AIR PERMEABLE FIBROUS BATT

Emanuel N. Maisel, Aurora, Ill., assignor, by mesne assignments, to Fiber Bond Corporation, Chicago, Ill., a corporation of Illinois

Application May 11, 1953, Serial No. 354,003

2 Claims. (Cl. 154—54)

This invention relates to an insulating batt of great resilience and loft, particularly suitable for use as an interlining for clothing, as an air or gas filter, and as a packing material for delicate objects.

This application is a continuation-in-part of my application Serial No. 290,481 filed May 28, 1952, now abandoned.

It is known that fibers may be formed into a self-supporting batt by coating the fibers with an adhesive which joins adjacent fibers of a batt. The fibers in this batt are assembled in layers with a random arrangement of fibers occurring substantially only within each layer. This batt maintains its resilience and loft for only a relatively short period of time when subjected to repeated rough handling, as when it is dry cleaned as a batt or is incorporated as an interlining in clothing which is dry cleaned. The dry cleaning chemicals and the high temperatures of the subsequent steam pressing of the clothes are also destructive of the batts made in accordance with the prior methods.

In accordance with the present invention the batts are made of non-matted, uncompressed fibers which are arranged randomly in three dimensions, namely, in all directions along the length, width and depth of the batt. The three-dimensionally-arranged fibers are non-matted and uncompressed and are held against matting and compression by a flexible adhesive, with the result that the batt has a softness, resilience and loft not heretofore attained in a batt. This batt has none of the disadvantages of the prior art batts. As hereinafter pointed out, it can be subjected to repeated dry cleaning and pressing operations without a breakdown of the arrangement of the fibers or a substantial loss in its original resilience and loft.

The batt constructed in accordance with the invention comprises a plurality of non-absorbent, non-matting fibers, preferably plastic fibers, either straight or curled, of various lengths of from about one half inch to two inches, held in three-dimensional, random, arrangement by means of a flexible adhesive. In making the batt, the individual fibers are first arranged in a three-dimensional, random arrangement and are then wetted lightly with adhesive to cause them to adhere to each other only at their spaced points of contact. The application of the adhesive and the drying thereof is effected without crushing or compacting the fibers of the batt. In consequence, the resulting batt is uncompressed and has an unusually high degree of softness and resilience and a very high loft. Although the batt may be handled and cut without any backing sheet, the application of a backing of cheese cloth or similar material facilitates such handling and cutting. The batt is capable of retaining stitches, and one or more batts may be stitched together, either with or without intervening sheets of cheese cloth or similar material, to form a batt of any desired thickness. When the batt is incorporated in a laminated fabric facing sheets may be stitched to both surfaces of the batt.

2

The adherence of the three-dimensional, randomly arranged fibers to each other at substantially only their points of contact imparts to the batt, and to laminated fabric in which the batt may be incorporated, excellent insulating and air retaining qualities. Air can pass readily through the batt, but only at a very slow rate, and the batt may be compressed, shaped around objects or cleaned without loss of softness, loft, or balling of the fibers.

Any adhesive which gives a flexible bond may be used in accordance with the present invention, but an elastic adhesive such as natural or synthetic rubber deposited from a latex emulsion is preferred. Where the batt is to be subjected to a dry cleaning operation, a synthetic rubber should be used. A suitable synthetic rubber is a vulcanizable, rubbery copolymer of butadiene and acrylonitrile, for example, that sold by B. F. Goodrich Co. under the trademark "Carbopol."

In accordance with the present invention, I have found that if the three-dimensional, randomly arranged fibers are of plastic material and are lightly wetted with a vulcanizable, synthetic rubber latex adhesive to adhere the fibers at the spaced points of contact, and the adhesive is then cured under controlled conditions, the resulting batt may be cleaned and steam pressed over and over again without loss, or without substantial loss, of softness, resilience or loft. In brief, the curing of the vulcanizable adhesive is effected by heating the adhesive coated batt to a temperature of from about 210° to 250° F., preferably about 220° to 230° F., for at least one minute. Although this curing temperature may be above the fusing temperature of the plastic fiber, surprisingly, the fiber does not undergo deterioration.

A preferred illustrative embodiment of an insulating batt and laminated fabric incorporating the above and other advantages is shown in the accompanying drawing, forming part of this specification, in which:

Figure 1 is a fragmentary plan view of the insulating batt incorporated into a laminated fabric, with portions broken away to show the laminated arrangement of different layers of material;

Fig. 2 is a fragmentary cross sectional view, taken along the line 2—2 of Fig. 1;

Fig. 3 is an enlarged detail view illustrating the three-dimensional, random arrangement of uncompressed fibers in the batt; and

Fig. 4 is a further enlargement of a portion of the fibers shown in Fig. 3, showing the fibers in a compressed state.

In the drawings, the reference numeral 2 indicates a batt of non-absorbent non-matting fibers 3. The fibers preferably are curled or crimped, but straight fibers of the same type may be used. The fibers may be natural fibers such as hogs hair, or they may be synthetic fibers such as nylon, rayon, acrylic fiber (a copolymer of vinyl chloride and acrylonitrile) commercially available under the trademark "Dyne," acrylic fiber (formed from a polymer of acrylonitrile) commercially available under the trademark "Orlon," or polyvinylidene chloride-polyvinyl chloride copolymer fiber commercially available under the trademark "Saran." Nonorganic fibers such as glass fiber, commercially available under the trademark "Fiberglas," may also be used. Any of these fibers may be used alone or mixed with each other.

The fibers are preferably of various lengths, from about one half inch to two inches, and are intermingled in random arrangement so that they lay at various angles, both horizontally and vertically, to form a three-dimensional batt with the individual fibers contacting each other at their separate points of contact throughout the batt. Relatively few pairs of individual fibers contact at more than one point, and each fiber of the batt contacts a

plurality of other fibers at spaced points which may be in the same or in different planes.

The batt is sprayed or otherwise coated lightly with an elastic adhesive on either one or both surfaces, preferably both surfaces. The amount of adhesive is sufficient to coat at least the outer fibers of the batt so that they adhere to each other and to the transversely extending fibers at their points of contact only, as indicated at 4. The spaces between the fibers should be substantially free of adhesive to maintain the softness and insulating properties of the batt. The small amount of the adhesive which passes through the interstices between the outer fibers wets the underlying fibers and causes them to adhere at their points of contact. The amount of adhesive applied is not sufficient to fill the voids between the fibers. Apart from incidental impregnation of some fibers with adhesive, the fibers are in the main unimpregnated and hence retain their natural springiness and impart to the batt the desired resiliency and loft.

The spaced joining of the three-dimensional, random arrangement of the fibers prevents matting and re-orientation of the fibers due to externally applied forces. Also, the elastic adhesive applied thereto substantially increases the resiliency of the batt.

The batts may be made of any desired thickness, say from three-eighths of an inch to two or more inches. When the batts are of about three-fourths of an inch or less in thickness, the fibers throughout the entire batt may be penetrated and coated with adhesive by a spraying operation applied to the outer surfaces thereof. It is not essential that the adhesive reach fibers in the center of the batt because the adhesive serves to tie the whole batt together by joining fibers extending transversely of the batt with the longitudinally extending fibers at both end portions of the transversely extending fibers.

Any elastic adhesive material such as natural rubber, synthetic rubber, or adhesive resinous or other plastic material may be used. Natural rubber, however, is not recommended when the end product in which the batt is incorporated is to be dry cleaned as it is attacked by the chemicals used in the conventional dry cleaning processes. When dry cleaning is contemplated, synthetic rubber should be used. The adhesive material may be applied in solution or in emulsion form. In the case of either natural or synthetic rubber, for example, it is applied in the form of an aqueous suspension or latex, with or without vulcanizing agents, and the adhesive coating is then dried to precipitate the rubber. Any conventional, commercially available, ammonium-stabilized, natural rubber latex may be used in accordance with my invention, alone or in combination with a synthetic rubber latex. A suitable synthetic rubber latex which may be used as the adhesive is the rubbery copolymer of butadiene and acrylonitrile sold under the trademark "Carbopol." If desired, there may be incorporated into the natural rubber latex or the mixed natural and synthetic rubber latex small amounts, about 0.25 to 3.0%, of a resin which serves to add quick tack and strength to the adhesive. Examples of resinous adhesives that may be used include solutions of polyvinyl chloride or polyvinyl acetate or copolymers thereof in organic solvents.

The adhesive applied to the fibers is dried to a non-tacky state, either naturally or artificially, without compacting the batt. This prevents the adhesive coating on any fiber from adhering to any other fiber except at the points where the fibers are in contact with each other in the uncompressed, three-dimensional, random arrangement in which the batt is initially formed. If the batt is compressed any time after the adhesive is dried, the fibers which are brought into contact by the compression will not adhere to each other, and the resiliency of the fibers will cause them to spring back to their original positions when the compressing force is released.

As previously stated, it is important that the random, three-dimensionally arranged fibers be adhered to each

other only at the points of contact to which the adhesive is originally applied. The adherence of the fibers to each other at their points of contact keeps the fibers in place and thereby maintains the loft and resiliency of the batt.

5 In Figs. 3 and 4 a plurality of random, three-dimensionally arranged fibers 3 are shown with adhesive 4 sheathing the fibers and adhering them together at their points of contact. The adhesive is dried in this position of the fibers. In Fig. 3 fibers of the batt are shown in their 10 normal uncompressed relationship and in Fig. 4 the same section of fibers is shown when the batt is temporarily compressed. As soon as the compressing force is released, the fibers shown in Fig. 4 will spring back to the positions shown in Fig. 3 because of the resiliency of the individual fibers and the elastic nature of the adhesive.

Where the batt is to be subjected to relatively high temperatures, as is the case where the batt is incorporated in articles which are steam pressed, the fibers of the batt may deteriorate to the extent that the batt loses its softness, resiliency and loft. Some of the synthetic fibers of the kind above described, such as "Dyne," for example, when subjected to temperatures above about 180° F., ordinarily begin to shrivel and lose their desirable properties. This action occurs even below the fusion point of 20 the fibers. When the fibers are raised to temperatures above the fusion point, the fibers of the batt fuse together and the batt completely loses its softness, resiliency, shape and loft. The temperatures utilized in conventional steam pressing operations are sufficiently high to deleteriously affect the relatively low melting point synthetic fibers such as "Dyne," except when they are properly protected in accordance with the present invention. Thus, 25 "Dyne" and like relatively low melting point plastic fibers may be protected against the deteriorating effects of 30 superheated steam such as is encountered in steam pressing operations, by the use of a vulcanizable synthetic rubber bonding medium which has been cured under 35 controlled conditions, as follows:

The batt of three-dimensional, randomly arranged 40 fibers having been lightly sprayed with a vulcanizable synthetic rubber latex, is carried into an oven on an endless carrier (not shown). Any source of dry heat may be applied to the batt in the oven, as for example the heat generated by a battery of infrared bulbs positioned 45 about one foot above the batt. The infrared bulbs supply heat in the region of the batt and throughout the batt. The heat of the batt should be raised to from about 210° to 250° F., preferably about 220° to 230° F., for at least about one minute, thereby effecting the 50 desired curing of the rubber. The curing of the rubber for longer periods of time, say two to five minutes, is not harmful. Nor is it necessary. One minute of time is generally adequate. During the curing operation, the water in the synthetic rubber latex is evaporated and the 55 desirable protective and adhesive properties of the synthetic rubber coating are developed. The drying oven, of course, should include air circulation to carry away the moisture accumulating therein.

One striking fact about the curing operation is to be 60 noted. "Dyne" fibers, for example, will ordinarily shrivel and otherwise deteriorate at temperatures above about 180° F. Yet, the very curing operation which is necessary to bring out the properties of the synthetic rubber coating which will protect the fibers against temperatures of 180° F. and above, is well above 180° F., namely, from 210° to 250° F., and the "Dyne" does not deteriorate.

Although the batt is preferably sufficiently thin that the sprayed adhesive will coat and sheath the fibers in 70 the center of the batt, it is not absolutely necessary to coat the batt fibers throughout the batt to protect the fibers in the central portion of the batt from the effects of high temperatures and dry cleaning. This protection is afforded by the outer coated fibers of the batt and by 75 the coated ends of the transversely extending fibers which

protect and insulate the uncoated fibers in the center of the batt and also tie them integrally into the batt.

The batt of the uncompressed, three-dimensional, randomly arranged fibers when formed is placed on the endless carrier which passes through the drying oven and the adhesive is applied to the batt, preferably as a spray, before the batt reaches the oven. The batt can be sprayed simultaneously from both sides thereof, a perforated endless carrier making this possible. It is preferred, however, to spray the adhesive initially only on the top surface of the batt and then carry the sprayed batt through the drying oven for curing of the adhesive. Thereafter, the batt is turned over and the uncoated side is sprayed with adhesive, and the twice coated batt is again passed through the drying oven to cure the freshly applied adhesive.

The batt formed as described above is uncompressed, yet is self-sustaining and has considerable strength in its lateral, longitudinal and transverse dimensions. It can be handled and be cut without the addition of any backing material and is capable of retaining stitches. The batt may be stitched directly to woven fabrics to form a laminated fabric.

The batt is an excellent air retainer and the insulating value thereof is very high. Because of the random, three-dimensional arrangement of the fibers, there are innumerable intercommunicating voids in the batt and air can pass through the batt, but only at a relatively slow rate. The batt can be compressed or cleaned without loss of loft or balling of fibers.

The resilience and loft retaining qualities of the batt are due primarily to the random, three-dimensional arrangement of the fibers, and to the thin, elastic adhesive coating which fastens the batt fibers together only at their spaced points of contact. The use of crimped or curled fibers increases the resilience of the batt over that attained with straight fibers. A cross section of a batt formed from crimped or curled fibers appears as a series of bridges in all directions and planes, thus giving greater loft than the same amount of straight fibers. The use of fibers of different lengths provides a better fiber distribution throughout the batt and also provides more points of contact.

When the batt is to be incorporated in a laminated fabric, facing sheets 5 and 7 are applied to opposite surfaces and secured to the batt by a line of stitching 8. If the batt is provided with a backing 6 of cheesecloth or similar material, the outer facing sheet, which is generally a woven fabric, is positioned adjacent backing sheet 6. The backing sheet imparts strength to the batt and aids in preventing the ends of the fibers of the batt from projecting through the interstices of the woven fabric. The laminated fabric is uniformly resilient throughout its area and does not require quilting to hold the fibers in sections.

The vast number of voids or air spaces in the batt imparts thereto such a high degree of porosity that the batt "breathes," and therefore it can be advantageously used as an interlining for garments or as an air filter. The batt conforms readily to the contours of irregularly shaped objects without loss of the cushioning properties of the batt and hence it is admirably suitable for use as a packing material, particularly for fragile and other readily breakable objects.

The importance of having a random, three-dimensional arrangement of uncompressed fibers cannot be overemphasized. The adhesive coated fibrous batting previously utilized included fibers arranged randomly generally along only two dimensions, that is in single planes or layers, and, in general, there was more or less of matting and compression of the fibers. In contrast, the arrangement of fibers which I use are random in all directions throughout the length, width, and depth of the batt, and there is no matting and compression of the fibers. There are innumerable fibers which extend transversely, i. e. 75

throughout the depth, of the batt and these fibers aid in tying the batt into an integral structure and in imparting to the batt its unusual properties of softness, resiliency and loft. By the term "random, three-dimensional arrangement" used in the claims and specification, is meant just such an arrangement of fibers as above described.

Although I have described a preferred embodiment of the invention in considerable detail, it will be understood that the description thereof is intended to be illustrative, rather than restrictive, as many details may be modified or changed without departing from the spirit or scope of the invention. Accordingly, I do not desire to be restricted to the exact structure and method described. For example, instead of applying the light adhesive coating to the fibers after they have been intermingled to form an uncompressed, three-dimensional, random arrangement of the fibers, the adhesive coating may be applied to the fibers before they are intermingled. The former procedure is the preferred procedure.

I claim:

1. An uncarded, uncompacted fibrous batt capable of passing air therethrough, said batt having a thickness up to about two inches, and a resilience and loft capable of being maintained on compression of the batt and subsequent release of pressure, said batt comprising a plurality of normally uncompressed plastic fibers of from about one-half inch to two inches in length, in intermingled, random, three-dimensional arrangement throughout the length, width and depth of the batt, there being individual fibers extending transversely throughout the depth of the batt to opposite upper and lower surfaces thereof and tying the batt into an integral structure from said upper and lower surfaces, said transversely extending fibers being bonded at spaced points to other fibers in the batt, a thin coating of a flexible adhesive about said transverse fibers and other fibers and throughout the batt, said adhesive bonding adjacent fibers in regions immediate their spaced points of contact, whereby the fibers are fixedly joined together at said spaced points to tie the batt into an integral structure, there being intercommunicating voids between the said fibers throughout the batt and no fibers in said voids, said voids being substantially free of adhesive, and said batt being of substantially uniform resilience and loft throughout.

2. An uncarded, uncompacted fibrous batt capable of passing air therethrough, said batt having a thickness from about one-half of an inch up to about two inches, and a resilience and loft capable of being maintained on compression of the batt and subsequent release of pressure, said batt comprising a plurality of normally uncompressed fibers of from about one-half inch to two inches in length, in intermingled, random, three-dimensional arrangement throughout the length, width and depth of the batt, there being individual fibers extending transversely throughout the depth of the batt to opposite upper and lower surfaces thereof and tying the batt into an integral structure from said upper and lower surfaces, said transversely extending fibers being bonded at spaced points to other fibers in the batt, a thin coating of a flexible adhesive about said transverse fibers and other fibers and throughout the batt, said adhesive bonding adjacent fibers in regions immediate their spaced points of contact, whereby the fibers are fixedly joined together at said spaced points to tie the batt into an integral structure, there being intercommunicating voids between the said fibers throughout the batt and no fibers in said voids, said voids being substantially free of adhesive, and said batt being of substantially uniform resilience and loft throughout.

**References Cited in the file of this patent****UNITED STATES PATENTS**

|           |                |               |
|-----------|----------------|---------------|
| 1,906,028 | Weber et al.   | Apr. 25, 1933 |
| 2,244,097 | Burkart        | June 3, 1941  |
| 2,418,904 | Rugeley et al. | Apr. 15, 1947 |
| 2,478,340 | Talalay        | Aug. 9, 1949  |
| 2,544,797 | Lippmann       | Mar. 13, 1951 |
| 2,550,465 | Górski         | Apr. 24, 1951 |
| 2,571,335 | Browne         | Oct. 16, 1951 |

|           |         |               |
|-----------|---------|---------------|
| 2,574,849 | Talalay | Nov. 13, 1951 |
| 2,580,202 | Talalay | Dec. 25, 1951 |
| 2,582,915 | Sebok   | Jan. 15, 1952 |
| 2,639,759 | Simison | May 26, 1953  |

**FOREIGN PATENTS**

|               |               |
|---------------|---------------|
| Great Britain | Jan. 26, 1931 |
| Great Britain | June 9, 1937  |
| France        | July 30, 1934 |